

United States Patent [19]  
Reznik

[11] 3,753,763  
[45] Aug. 21, 1973

[54] COATINGS FOR COLUMBIUM AND  
COLUMBIUM BASE ALLOYS

[75] Inventor: Barry D. Reznik, Brooklyn, N.Y.

[73] Assignee: The United States of America as  
represented by the Atomic Energy  
Commission, Washington, D.C.

[22] Filed: Jan. 24, 1964

[21] Appl. No.: 340,112

[52] U.S. Cl..... 117/62, 29/195, 29/197,  
29/198, 29/199, 117/71, 117/104 R, 117/105,  
117/127, 117/130 R, 117/135.1

[51] Int. Cl. .... C23f 14/00, C23b 11/00, B23p 3/20

[58] Field of Search..... 117/104, 105, 127,  
117/130, 104 R, 130 R, 135.1, 71, 62 R;  
29/195, 197, 198, 199

[56] References Cited

UNITED STATES PATENTS

3,317,343 5/1967 Jefferys ..... 117/130 R  
3,294,497 12/1966 Foldes et al. ..... 29/194 X

3,293,068 12/1966 Bradley et al. .... 117/127 X  
2,763,919 9/1956 Kempe et al. .... 29/198 X

Primary Examiner—Carl D. Quarforth

Assistant Examiner—Roger S. Gaither

Attorney—Roland A. Anderson

[57] ABSTRACT

A method of protectively coating columbium and columbium-base substrates for service at temperatures above 2000° F comprising spray coating the substrate with a slurry consisting of a powdered mixture of silicon, aluminum and silver in a lacquer followed by diffusion treating the coated substrate in an inert atmosphere at a temperature in the range of 1900° F to 2300° F to form a layer of silicide intermetallic compounds adjacent the substrate and a layer of silver-silicon-aluminum alloy overlaying the first layer.

9 Claims, 3 Drawing Figures

PATENTED AUG 21 1973

3,753,763



FIG. 1



FIG. 2



FIG. 3

INVENTOR.

BY BARRY D. REZNIK

*Barry D. Reznik*  
Attorney

## COATINGS FOR COLUMBIUM AND COLUMBIUM BASE ALLOYS

This invention relates generally to the field of metallurgy and is directed in particular, to a new method of protectively coating columbium and columbium alloys against oxidation at temperatures of 2,000°F and above, together with the article produced thereby.

Columbium and its alloys possess a unique balance of properties that make their use particularly attractive for high temperature space and nuclear applications. Where any of these applications require resistance to oxidation, however, protective coatings must be used, and their development has been vigorously pursued for a number of years.

Heretofore protective coatings for columbium and its alloys have been successfully developed which will provide short time protection of from minutes to a maximum of about 100 hours at temperatures up to about 2,600°F. The most successful of these coatings have been obtained by pack coating with a mixture of titanium-chromium and silicon, or by slurry coating with a tin-aluminum alloy.

The foregoing coating methods, while suitable for some applications, are unsatisfactory from certain points of view. For example, the tin-aluminum slurry coatings of the prior art can not be relied upon for prolonged protection at 2,000°F since it has been found that at this temperature the aluminum in the coating diffuses into the substrate and combines to form  $\text{Cb}_2\text{Al}$ . This gradually removes aluminum from the coating and leads to failure in the course of time at 2,000°F. At higher temperatures, such as 2,500°F and above, the tin-aluminum base coatings have no useful life on columbium or columbium base alloys.

The Ti-Cr-Si coating, although effective in its ability to protect columbium substrates from oxidation, is both expensive and time consuming to apply since it requires multicycle high-temperature vacuum heating treatments. Additionally, the high temperatures employed in the coating process has an adverse effect on the mechanical properties of the substrate.

It is the object of this invention to provide a new method of coating columbium and columbium base alloys so as to protect the columbium against oxidation at temperatures of approximately 2,000°F for at least a period of hundreds of hours. It is a further object to provide a coating that is readily and economically applied to the columbium or columbium base alloy and which can be applied without adversely affecting the mechanical properties of the columbium.

The foregoing objects are achieved by coating the columbium with alloys of silver and silicon or of silver, silicon and aluminum. Thereafter the coated article is given a diffusion treatment in a vacuum or in argon to form a coating consisting of a layer of silicide intermetallic compounds adjacent the substrate, over which is a layer of the silver-silicon base alloy.

The invention may be more completely understood by reference to the figures, wherein

FIG. 1 is a photomicrographic (300x) of columbium coated with an alloy consisting of Ag-10 Si - 1 Al in accordance with this invention.

FIG. 2 is a photomicrograph (300x) of a specimen as in FIG. 1 after exposure for 100 hours at 2,500°F., and

FIG. 3 is a graph comparing the oxidation life of an Ag-15 Si-1 Al coating with a Ti-Cr-Si coating on columbium under cyclic conditions at temperatures between 2,600°F and 3,000°F.

The coatings of the present invention are prepared by first suitably cleaning the substrate in any suitable manner, such as by blasting with angular steel grit.

Next, the substrate is coated by cold spraying with a slurry made up of a mixture of fine (minus 300 mesh) silver, silicon and/or aluminum metal powders with an equal volume of lacquer. After air drying, the sample is given a diffusion treatment in a vacuum or in an argon atmosphere for periods of from 10 to 15 minutes at temperatures in the range of 1,900°F to 2,500°F., to form a coating consisting of a layer of silicide intermetallic compounds, presumably  $\text{Cb Si}_2$ , adjacent the substrate. Overlying the silicide layer is an outer layer of a Ag-Si-Al alloy, as may be seen by inspection of FIG. 1.

After oxidation for 100 hours at 2,500°F a specimen as in FIG. 1, retains a protective coating, as shown in FIG. 2. It is important to note that the inward diffusion of the coating into the substrate is slow; amounting to only 1.25 mil penetration after 100 hours at 2,500°F. Metallographic studies of samples oxidized at 2,000°F show that the rate of conversion of  $\text{CbSi}_2$  to  $\text{Cb}_5\text{Si}_3$  is slow and would require 6,000 hours at that temperature to convert a coating containing a thickness of 1 mil  $\text{CbSi}_2$  to  $\text{Cb}_5\text{Si}_3$ . It is therefore apparent that this coating, applied in suitable thickness can achieve the desired goal of protection for the desired period of 2,000°F.

It has been observed that no one coating is equally protective to all columbium alloys, and that with the development of each new alloy one must either reevaluate or modify an existing coating or develop an entirely new coating in order to provide the required oxidation protection. Because of this unpredictability in the behavior of columbium and its alloys, experiments were conducted with columbium, and two columbium-base alloys identified respectively as X-110 (Cb-10W-1 Zr-0.6C) and B-66 (Cb-5Mo-5V-1 Zr). The latter two alloys are of interest because of their superior mechanical properties as compared, for example, with an alloy such as Cb-1 Zr, and coupled with their good fabricability. Results of preliminary screening tests are given in the following Table I. In each instance, the diffusion step was repeated to increase the thickness of the coating:

TABLE I  
Oxidation Protectiveness of Ag-Si Base Slurry Coating

| Sample No. | Base alloy | Coating composition | Diffusion treatment | Oxidation life (hours) |           |             |
|------------|------------|---------------------|---------------------|------------------------|-----------|-------------|
|            |            |                     |                     | 1,100° F.              | 2,000° F. | 2,500° F.   |
| B21-47-1   | Cb         | Ag-25Si             | A                   | 100                    | 100       | 50 19       |
| B21-47-6   | Cb         | Ag-17Si             | A                   | 200                    | 175       | 260 100     |
| B102-36-1  | Cb         | Ag-10Si             | B                   | 1,000                  | 110       | 196 75 83   |
| B102-46-1  | Cb         | Ag-10Si-1Al         | A                   | ND                     | 200       | 300 105 100 |
| B102-46-11 | Cb         | Ag-10Si-5Cr-1Al     | A                   | 180                    | 100       | 200 30 40   |
| B102-46-19 | Cb         | Ag-10Si-5Cr-5Ti     | A                   | 660                    | 100       | 200 22 27   |

TABLE I  
Oxidation Protectiveness of Ag-Si Base Slurry Coating

| Sample No. | Base alloy | Coating composition | Diffusion treatment | Oxidation life (hours) |           |           |
|------------|------------|---------------------|---------------------|------------------------|-----------|-----------|
|            |            |                     |                     | 1,100° F.              | 2,000° F. | 2,500° F. |
| B102-32-1  | Cb         | Ag-15Si-5Cr         | A                   | 470                    | 800       | 150       |
| B102-31-11 | Cb         | Ag-15Si-1Al         | A                   | 150                    | 500       | 100       |
| B102-52-1  | Cb         | Ag-10Si-1Al         | B                   | 610                    | 700+      | 100       |
| B102-52-11 | B-66       | Ag-10Si-1Al         | B                   | 400                    | 680       | 60        |
| B102-52-21 | X-110      | Ag-10Si-1Al         | B                   | 350                    | 350       | 122       |
| B102-54-1  | Cb         | Ag-10Si-1Al         | C                   | 60                     | 60        | 30        |
| B102-60-1  | Cb         | Ag-15Si-1Al         | B                   | -----                  | ND        | 255       |
| B102-60-6  | Cb         | Ag-15Si-3Al         | B                   | -----                  | ND        | 315+      |
| B102-60-11 | Cb         | Ag-15Si-5Al         | B                   | -----                  | ND        | 315+      |
|            |            |                     |                     |                        |           | 50        |
|            |            |                     |                     |                        |           | 50        |

NOTE.—Diffusion treatment:

A=double diffusion 10 minutes at 2,300° F. in argon,  
B=double diffusion 15 minutes at 2,300° F. in argon,  
C=double diffusion 15 minutes at 1,900° F. in vacuum.

ND=Not determined.

As diffusion treatments in vacuum result in substantial losses of Ag by volatilization, it is deemed preferably to employ an argon atmosphere at 1 atmosphere pressure to minimize such losses.

The effectiveness of the Ag-Si-Al coating on pure columbium under cyclic oxidation conditions at temperatures of 2,600°F and above is shown in FIG. 3 which shows that this coating has twice the effective life at 3,000°F as the best known coating, Ti-Cr-Si.

Subsequent tests illustrating the effectiveness of the Ag-Si-Al coatings on B-66 and X-110 alloys are summarized in the following Table 2. The findings listed in the following Table 2 also show the value of preoxidation of the coated sample in increasing oxidation resistance at temperatures of 1,100°F and 1,800°F. In the examples given in the table, the preoxidation step was conducted in air at about 2,500°F for a period of 2 hours and resulted in a substantial increase in low temperature resistance of the samples.

also permits the oxide film to grow on the liquid, thereby eliminating stresses between the surface oxides and the intermetallic compounds.

- 20 It has been observed that the best coatings for service at temperatures of 2,500°F and above are the Ag-15 Si-1Al coatings, as illustrated in FIG. 3. However, for use at 2,000°F coatings of Ag-15 Si-7.5 Al and Ag-15 Si-8 Al give the best results. It is believed that at the lower temperature greater amounts of aluminum are useful in preventing loss of Ag by volatilization.  $Al_2O_3$  forms preferentially on oxidation at 2,000°F. As loss of Ag through  $Al_2O_3$  is slow, the sample initially gains weight as the  $Al_2O_3$  forms. As oxidation progresses,  $SiO_2$  also forms and grows. At the same time the concentration of  $Al_2O_3$  decreases to a point where it becomes permeable to the Ag. Thereafter, loss of Ag exceeds the rate of oxidation of the sample, and the latter loses weight.
- 25 Hence, the higher the aluminum concentration the
- 30
- 35

TABLE 2

| Sample      | Base alloy | Coating composition (w/o) | Oxidation life, hours |           |           | Samples preoxidized 2 hrs., 2,500° F. |           |
|-------------|------------|---------------------------|-----------------------|-----------|-----------|---------------------------------------|-----------|
|             |            |                           | 1,100° F.             | 1,800° F. | 2,000° F. | 1,100° F.                             | 1,800° F. |
| B-102-82-1  | Cb         | Ag-15Si-1Al               | 200                   | 477       | 200       | 590                                   | 700       |
| B-102-82-9  | Cb         | Ag-15Si-3Al               | 200                   | 66        | 200       | 608                                   | 650       |
| B-102-82-17 | Cb         | Ag-15Si-5Al               | 200                   | 200       | 270       | 300                                   | 1,000     |
| B-102-86-1  | B-66       | Ag-15Si-1Al               | 245                   | 630       | 690       | 585                                   | 860       |
| B-102-86-9  | B-66       | Ag-15Si-3Al               | 245                   | 175       | 680       | 680                                   | 730       |
| B-102-86-17 | B-66       | Ag-15Si-5Al               | 175                   | 175       | 800       | 460                                   | 525       |
| B-102-88-1  | X-110      | Ag-15Si-1Al               | 240                   | 300       | 580       | 235                                   | 235       |
| B-102-88-9  | X-110      | Ag-15Si-3Al               | 175                   | 175       | 410       | 235                                   | 235       |
| B-102-88-17 | X-110      | Ag-15Si-5Al               | 67                    | 245       | 630       | 235                                   | 235       |
| B-277-6-10  | Cb         | Ag-15Si-7.5Al             | ND                    | -----     | 1,720     | 1,750+                                | ND        |
| B-277-8-1   | Cb         | Ag-15Si-5Al               | ND                    | ND        | 875       | 875                                   | ND        |
| B-277-8-4   | Cb         | Ag-20Si-7Al               | ND                    | ND        | 800       | 1,030                                 | ND        |
| B-277-8-7   | Cb         | Ag-15Si-7.5Al             | ND                    | ND        | 1,150     | 1,270                                 | ND        |
| B-277-8-11  | Cb         | Ag-25Si-8Al               | ND                    | ND        | 910       | 1,030                                 | ND        |
| B-277-7-1   | Cb         | Ag-15Si-5Al               | -----                 | -----     | 875       | 875                                   | -----     |
| B-277-7-4   | Cb         | Ag-20Si-7Al               | -----                 | -----     | 800       | 1,030                                 | -----     |
| B-277-7-7   | Cb         | Ag-25Si-8Al               | -----                 | -----     | 910       | 1,030                                 | -----     |
| B-277-6-7   | Cb         | Ag-15Si-8Al               | -----                 | -----     | 1,780     | 2,000+                                | -----     |

NOTE.—ND=Not Determined.

Useful coatings may be obtained in the range of 3 to 30 w/o Si and 1 to 10 w/o Al, the balance being Ag. However, it is to be noted from the results tabulated in the foregoing Table 2, that for service at 2,000°F, the longest oxidation life was achieved with a slurry consisting of Ag-15 Si-7.5Al.

It has been found that the aluminum is useful in improving the low temperature and thermal cycle capabilities of this coating. In contrast, additions of Cr and Ti have been shown to be detrimental.

While the reason for the effectiveness of the present coating is not completely understood, it is apparent that liquid silver-silicon base alloy acts as a reservoir for repairing defects in the surface oxide film, and it

55 longer it takes for losses of Ag to assume significant proportions. At temperatures of 2,500°F and above, however, a different mechanism appears to be operative since it has been observed that concentrations in excess of 1 w/o Al actually decrease the oxidation life 60 of the sample. It is believed that this decrease in oxidation life results from the formation of lower melting point oxidation products at this temperature.

From the foregoing it will be seen that useful coatings for columbium and columbium base alloys have been produced which will protect the base metal against oxidation at temperatures of 2,000°F and above for useful periods of time.

I claim:

1. The method of protectively coating columbium and columbium-base substrates for service at temperatures of 2,000°F and above that consists of the steps of:
  - a. Cleaning the substrate;
  - b. Preparing a powdered material consisting of silver, silicon and aluminum powders in the following proportions by weight: 3 to 30 percent silicon; 1 to 10 percent aluminum and the balance silver;
  - c. Preparing a slurry by suspending said material in a lacquer;
  - d. Spray coating the substrate with the slurry; and
  - e. Diffusion treating the coated substrate in an inert atmosphere at a temperature in the range of approximately 1,900°F to 2,300°F to form a layer of silicide intermetallic compounds adjacent the substrate and a layer of silver-silicon-aluminum alloy overlying the said silicide intermetallic compounds.
2. The method of claim 1 wherein the powdered material consists of 15 per cent by weight silicon, 8 per cent by weight aluminum and the balance silver.
3. The method of claim 1 wherein the coated sample is preoxidized in air at a temperature of approximately 2,500°F following diffusion treatment to improve oxidation resistance of the sample.

4. The method of claim 1 wherein the columbium-base alloy has the following composition by weight per cent:

5 Cb - 5 Mo - 5V - 1Zr.

5. The method of claim 1 wherein the columbium-base alloy has the following composition by weight per cent:

10 Cb - 10W - 1 Zr - 0.6C.

6. A columbium substrate having an oxidation protective coating thereon said coating consisting of a silicide intermetallic layer on the substrate and a silver-silicon-aluminum alloy layer on the said intermetallic 15 layer.

7. The article of claim 6 wherein the substrate consists of a columbium base alloy having the following composition by weight:

20 Cb - 5 Mo - 5 V - 1 Zr.

8. The article of claim 6 wherein the substrate consists of a columbium-base alloy having the following composition by weight:

25 Cb - 10W - 1 Zr - 0.6C.

9. The article of claim 6 wherein the silicide intermetallic layer has the approximate composition: Cb Si<sub>2</sub>.

\* \* \* \* \*

30

35

40

45

50

55

60

65